

Patented Nov. 30, 1926.

1,608,501

# UNITED STATES PATENT OFFICE.

FRANK J. GRISWOLD, OF PORT CLINTON, OHIO, ASSIGNOR TO THE AMERICAN GYPSUM COMPANY, OF PORT CLINTON, OHIO, A CORPORATION OF OHIO.

## METHOD OF MANUFACTURING PLASTER BOARD.

No Drawing.

Application filed July 27, 1923. Serial No. 654,235.

This invention relates to improvements in method of manufacturing plaster board and more particularly to a novel process of treating the materials during the manufacturing of the product to secure better and more uniform quality.

Plaster board is a well known building material, consisting in its most common form, of a layer of stucco or plaster interposed between covering sheets of a suitable grade of paper. Plaster board is manufactured commercially by machinery designed to produce the board by a continuous process whereby the paper is fed from rolls into the machine, the stucco in a plastic state introduced between the sheets and the assembled materials passed between forming rolls which reduce the product to a uniform thickness. The board in its wet state is then carried for a distance on a horizontal conveyor to give the stucco an opportunity to set, and is then cut into sheets of convenient size, and finally dried in kilns.

The foregoing brief description of the process of manufacture does not take into consideration the difficulties that are encountered, due to the irregularities in quality and condition of materials. In the first place, the problem of adhesion between the paper and stucco is a difficult one to control. Under ideal conditions this would be satisfactorily accomplished by a partial saturation of the paper by the moisture in the stucco and the formation of a natural bond between the surfaces. However, it is a difficult matter to regulate the amount of saturation or quantity of moisture in the stucco for the reason that the paper supply is seldom of a uniform quality,—different grades or variations in the treatment of the paper having a marked effect on the properties of the paper to absorb moisture. If the paper absorbs the moisture readily, there is a possibility of over-saturation and a weakening of the paper structure. On the other hand, under-saturation results in poor adhesion between the materials. Either condition is detrimental to the finished board, since over-saturation produces a weak product, and under-saturation produces an ineffective bond, with the result that the paper peels from the stucco after the board is dried so that it is either useless or of a very inferior grade.

The purpose of this invention is there-

fore to devise a method of treating the materials, preferably the surface of the paper, in such a way as to eliminate all uncertainties of quality and conditions, by providing a mechanical adhesion or bond between the surface of paper and stucco that will be uniform and effective, thus making it possible to produce a superior product without loss, and of increased strength.

In a few words the process consists of applying a water-resisting and adhesive composition to the surface of the paper coming into contact with the stucco, the application being preferably made as the paper is fed from the rolls and dried, before contact with the stucco takes place. The result of treating the surface of the paper is twofold; first, the surface of the paper is waterproofed thereby reducing the subsequent saturation of the paper; and second, to supply the adhesive substance made necessary by the elimination of the natural bond by the water-resisting means.

While numerous compositions may be found suitable for this purpose, experiment has revealed the fact that a solution of gum arabic or acacia, aluminum sulphate and water provides a very satisfactory composition for this purpose. The solution preferably consists of 5% each of gum arabic and aluminum sulphate dissolved in 90% of water, although this proportion may be varied somewhat without affecting the properties of the solution.

The method of application may be varied to meet different operating conditions, but on the whole, a very satisfactory method is to spray the solution onto the surface of the paper. This can be readily accomplished by suitable atomizing or spraying nozzles directed toward the paper as it leaves the roll, although any means which will spread a thin coating of the liquid composition uniformly over the surface of the paper would be quite as satisfactory.

The drying of the composition after its application and before the paper comes into contact with the wet stucco is obviously a matter of driving off the water content of the solution within the shortest space of time permitted by the distance and rate of travel of the paper from the roll to the point of contact with the stucco. The use of either steam coils or fans, or both, will be found to be quite satisfactory. If steam coils are

used they would be located in the path of the paper just beyond the point of application of the waterproofing composition, and in close proximity to the surface so that in passing over the coils the heat effectively dries the coating. Similarly the fans would be mounted to direct a current of air against the surface of the paper as it advances toward the machine, and where both steam coils and fans are used, the fans would direct the current of air through the coils and against the surfaces to be dried. Since there are ordinarily two surfaces to be coated, namely, the inner surface of the top and bottom sheets, the composition applying and drying devices may be arranged to care for both or separate devices provided for each sheet.

Subsequent to the drying process, the paper is brought into contact with the wet stucco, and passed through the rolls in the usual manner. It follows that the coating is again moistened to create the adhesion or bond between the surfaces of paper and stucco which becomes permanent when the board is subsequently dried.

Under some conditions the process may include the sprinkling of fine sand or other pulverized substance over the surface to which the adhesive composition has been applied, and before it is dried. This material affords a roughened surface and therefore a more complete bond between the paper and the stucco.

By the treatment of the paper with a coating of a composition such as herein set forth, a mechanical bond is established between the materials which is not dependent on the quality of the paper or upon the amount of moisture contained in the stucco in order to secure effective adhesion between the surfaces. This feature of the process, therefore, suggests that different grades of paper can be used without considering its ability to adhere to the stucco thus widening the range of materials available for making the product.

While a specific process of treatment has been herein described it is manifest that the same results can be obtained with other compositions and with different methods of application. As an example the paper might be readily treated by the paper manufacturer and shipped to the plaster board manufacturer ready for use. For these reasons it is not the intention to limit the invention to the particular method or methods herein disclosed.

I claim as my invention:

1. A process of manufacturing plaster board consisting of treating the inner surfaces of the covering material with a liquid composition of gum arabic and aluminum sulphate and introducing stucco in its wet state between sheets of said covering material.

2. A process of manufacturing plaster board consisting of treating the inner surfaces of the covering sheet as it is fed from a roll with a coating of a liquid composition of gum arabic and sulphate of aluminum, drying the coating by the application of heat or air, and introducing stucco in its wet state between the sheets.

3. A process of manufacturing plaster board consisting of spraying the inner surfaces of the sheets of covering paper with a solution of substantially five percent (5%) each of gum arabic and aluminum sulphate dissolved in water, drying the sheets and then introducing stucco between said sheets.

4. A process of manufacturing plaster board consisting of spraying the inner surfaces of the covering sheets as they are fed from the rolls, with a solution of 5% of gum arabic and 5% of sulphate of aluminum dissolved in 90% of water, drying the surfaces of the sheets by the application of heat or air, or both, and introducing stucco in its wet state between the sheets, subsequent to the drying process.

In witness whereof, I hereunto subscribe my name this 24th day of July, A. D. 1923.

FRANK J. GRISWOLD,